

## UNITED STATES PATENT OFFICE

2,539,907

DYED CARROTED FUR FIBERS AND FABRICS  
AND METHOD OF DYEING THE SAMEStanley G. Hoffman, Norwalk, Conn., assignor to  
Hat Corporation of America, Norwalk, Conn., a  
corporation of DelawareNo Drawing. Application April 14, 1948,  
Serial No. 21,096

5 Claims. (Cl. 8—26)

1

The present invention relates to dyed fur fibers, dyed fur felt fabrics or hat bodies and the method of producing the same.

Mottle or ununiform color appearing in fur felt hats has been a problem in the fur felt industry for over one hundred years. This mottle usually shows up to a greater degree the more the hats or fabrics are processed to remove the rough outer surface and produce a finer felt so that a great loss both as to time and acceptable product is sustained. The presence of mottle in the fabric has been attributed to many factors. Some believed that it was due to the condition of the animal when the fur was taken, others believed that it was due to the working of the felt into fabric form and still others believed that it was due to poor dye penetration.

While many attempts have been made to overcome this condition, such as more careful selection and combining of the fur fibers, variations in the treatment of the fur during felting and in the dye cycle, these efforts have been ineffective to overcome this defect.

I have discovered that the cause of mottle does not reside in the factors noted above, but instead is caused by the fact that the fur fibers when dyed with the usual acid dye for fur did not dye uniformly throughout the length thereof and that this condition resulted from a changing of the tip portion of the fibers during the carroting operation to which they are subjected to improve the felting properties of the fur fiber, and that the amount of mottle bears a definite relation to the extent of carroting of the fibers in the fabric. In other words, if a fur is given a light carroting treatment, a lesser amount of the tip is changed and a minimum of mottle is produced. If the fur is subjected to a strong carroting operation a greater amount of the fiber is changed chemically and physically and a greater amount of mottle appears in the fur fabric.

In the carroting operation, the fur fibers are treated by brushing with a carroting solution which may be either of the mercuric or non-mercuric type. This treatment softens the tips and causes the fibers to felt together better. The term "carroted fur" as used herein designates such fibers.

In softening the tips, the carroting treatment changes the fur in the tips both chemically and

2

physically. I have found that this change in the tips causes them to have a less affinity for the usual acid dye than the remainder or stems of the fibers. Thus each carroted fiber when dyed with acid dye would have the required color on the stem but much less or no color on the tip. When these fibers are felted to form the fabric the lesser dyed or undyed tip portion which usually works to the center of the felt produces the light spots in the dyed fabric.

This difficulty has been overcome according to the present invention by dyeing the fabric, hat body and/or fibers with a combination of dyestuffs which dye both the tip and stem substantially the same amount so as to produce a uniform or level color throughout the fiber.

I have found that an acid metallized dyestuff, i. e., an acid dyestuff which is a metal compound of azodyestuff, as for example described in U. S. Patent No. 1,753,120, has a strong affinity for the carroted tip and a much less affinity for the stem of the fiber. The acid metallized dyestuff differs from the conventional mordant dyestuffs which usually require the addition of mordant at the start of dyeing or as an after-treatment. When this dyestuff is used alone there is a tendency to produce a shadow effect or reverse mottle. However, when it is combined with an acid dyestuff normally used for dyeing fur felt, and for which the stem of the fur fiber has a strong affinity, in proper proportions as determined by the extent of the carroting operation, a uniform color on the fiber and elimination of mottle from the fabric or hat body, even when the fabric and/or hat body are processed to produce a fine finish, is obtained.

In ascertaining the proportions of the acid dyestuff and acid metallized dyestuff to be used in the combination, the fur to be dyed is tested by the usual felting test to determine the extent of the carroting action. After the extent of carroting action has been determined the amount of acid metallized dye necessary to color the tip and the amount of acid dye to color the stems can be readily determined by those skilled in the art.

The acid dyes used in accordance with the present invention are any of the known acid dyes now used for dyeing fur. The acid metallized dyes for dyeing the tips may be any of the known

metallized dyes having an affinity for the carotted tips of the fur fiber.

For example, a blue dye of this class may be selected from those indicated under Color Index, Prototype #144 as follows:

Amalan Blue GGL  
Calcofast Wool Blue 2G  
Chromolan Blue NGG  
Chromacyl Blue GG  
Gycolan Blue GGL  
Neolan Blue GG  
Nyasol F. Blue 2GA  
Palatine Fast Blue GGNA  
Vitrolan Blue 2G

I have also found that the Palatine dyes produced by General Dyestuff Corporation are particularly satisfactory for this purpose. Such dyes are:

Palatine Fast Black WANA Conc. (C. I. Pr. 143)  
Palatine Fast Blue BNOA (C. I. Pr. 318)  
Palatine Fast Blue GGNA (C. I. Pr. 144)  
Palatine Fast Blue RRNA (C. I. Pr. 319)  
Palatine Fast Claret BNA (C. I. Pr. 394)  
Palatine Fast Claret RNA Conc. (C. I. Pr. 320)  
Palatine Fast Green BLNA Conc. (C. I. Pr. 321)  
Palatine Fast Marine Blue RENA (C. I. Pr. 322)  
Palatine Fast Orange GEN (C. I. Pr. 323)  
Palatine Fast Orange GNA (C. I. Pr. 324)  
Palatine Fast Pink BNA (C. I. Pr. 326)  
Palatine Fast Palatine Red RNA (C. I. Pr. 327)  
Palatine Fast Violet 3 RNA (C. I. Pr. 328)  
Palatine Fast Violet 5 RNA (C. I. Pr. 329)  
Palatine Fast Yellow ELNA (C. I. Pr. 330)  
Palatine Fast Yellow GRNA (C. I. Pr. 331)

If the desired color or shade is not available, two or more metallized dyes are blended to produce the required color and two or more of the acid dyes are blended to produce the desired color. The proportion of the weight of each of the blended acid metallized and acid dyes corresponding to the required proportion as determined by the tests are then mixed in water with a small amount of glauber salt and sulphuric acid to provide the dye bath for the fabric or hat bodies. The hat body or fabric is immersed in the bath which is at a temperature of approximately 120° and the bath is then brought to a higher temperature or to boiling and the material maintained therein for about one hour or more after which it is removed and the fabric processed in the usual manner.

For example, in dyeing one lot of hat bodies a Fawn Brown, it was determined that the combination of dyes should include 30% acid metallized dyes and 70% of acid dyes. To produce the required color, the following acid metallized dyes and acid were combined.

| Acid Metallized Dyes     | Per Cent of Weight of Material Dyed | Acid Dyes               | Per Cent of Weight of Material Dyed |
|--------------------------|-------------------------------------|-------------------------|-------------------------------------|
| Chromolan Blue NGG       | 0.15                                | Alizarine Fast Blue KFG | 0.36                                |
| Palatine Fast Orange GEN | 0.70                                | Tartrazine              | 0.19                                |
| Chromolan Yellow NGR     | 0.24                                | Wool Orange 2G          | 0.22                                |
| Palatine Fast Pink BNA   | 0.16                                | Fast Crimson 6BL        | 0.09                                |

These were dissolved in water and to the dyeing solution was added 10% of weight of material dyed of glauber salt and 3% of weight of material dyed of sulphuric acid. The hat bodies

75

were placed in the dye and dyed in accordance with the procedure outlined above.

In another example, a group of hat bodies were to be dyed a color Vista (a blue-gray). It was determined that the combination should include 70% metallized dyes and 30% acid dyes. To produce the required color, the following acid metallized dyes and acid dyes were combined.

| 10 | Acid Metallized Dyes     | Per Cent of Weight of Material Dyed | Acid Dyes               | Per Cent of Weight of Material Dyed |
|----|--------------------------|-------------------------------------|-------------------------|-------------------------------------|
| 15 | Chromolan Blue NGG       | 0.31                                | Alizarine Fast Blue KFG | 0.14                                |
|    | Palatine Fast Orange GEN | 0.24                                | Erio Brown 5RL          | 0.08                                |
|    | Palatine Fast Yellow ELN | 0.18                                | Fast Light Yellow 3G    | 0.01                                |
|    | Palatine Fast Pink BNA   | 0.28                                | Azo Rhodine 2G          | 0.045                               |

20

These were dissolved in water and to the dyeing solution was added 10% of weight of material dyed of glauber salt and 3% of weight of material dyed of sulphuric acid. The hat bodies were placed in the dye and dyed in accordance with the procedure outlined above.

In still another example, a group of hats were to be dyed Nickel Grey. It was determined that the combination should include 50% metallized dyes and 50% acid dyes. To produce the required color, the following acid metallized dyes and acid dyes were combined.

| 35 | Acid Metallized Dyes     | Per Cent of Weight of Material Dyed | Acid Dyes          | Per Cent of Weight of Material Dyed |
|----|--------------------------|-------------------------------------|--------------------|-------------------------------------|
| 40 | Chromolan Blue NGG       | 0.15                                | Alizarine Blue KFG | 0.20                                |
|    | Palatine Fast Orange GEN | 0.30                                | Erio Brown 5RL     | 0.18                                |
|    | Palatine Fast Yellow ELN | 0.07                                | Azo Rhodine 2G     | 0.03                                |
|    | Palatine Fast Pink BNA   | 0.08                                |                    |                                     |

50

These were dissolved in water and to the dyeing solution was added 10% of weight of material dyed of glauber salt and 3% of weight of material dyed of sulphuric acid. The hat bodies were placed in the dye and dyed in accordance with the procedure outlined above.

While it is at present preferred to dye the fur fibers after they have been felted into a fabric or a hat body, it is to be understood that loose carotted fur fibers may be dyed with the combined dyestuffs.

The tips and stems may be dyed in separate operations but it is at present preferred to mix the acid and acid metallized dyes in a single bath and dye the fibers in a single operation. The dyestuff may be mixed by the user as required. However, it is to be understood that it may be also compounded by the dyestuff manufacturer to include the acid dyestuff and acid metallized dyestuff in the proportions most generally used by the hat manufacturers and sold to the hat manufacturers in this form.

Variations and modifications may be made within the scope of this invention and portions of the improvements may be used without others.

I claim:

1. A carotted fur fiber dyed a level color with the tip portion dyed with an acid metallized dye and the remainder dyed with an acid dye of similar color.
2. A carotted fur fiber dyed in level color with

an acid metallized dye and an acid dye of similar color.

3. A mottle-free fabric of felted carotted fur fibers dye with an acid metallized dye and acid dye of similar color.

4. A mottle-free hat body of felted carotted fur fibers dyed with an unreacted mixture of an acid metallized dye and acid dye of similar color.

5. The process of dyeing a felt hat body of carotted fur fibers comprising preparing a dye bath including a mixture of acid dyestuffs and acid metallized dyestuffs of similar color; immersing the hat body in the bath; and maintaining the hat body in the bath until the required shade is obtained.

STANLEY G. HOFFMAN.

#### REFERENCES CITED

The following references are of record in the file of this patent:

#### UNITED STATES PATENTS

| Number    | Name   | Date          |
|-----------|--------|---------------|
| 1,887,603 | Straub | Nov. 15, 1932 |

#### FOREIGN PATENTS

| Number  | Country       | Date           |
|---------|---------------|----------------|
| 526,760 | Great Britain | Sept. 25, 1940 |

#### OTHER REFERENCES

Textile Colorist, for April 1943, pages 177, 178, 179.

15 "Jour. Soc. Dyers and Chem.," for June 1944, pages 144, 145 (article by Townsend).

"Amer. Dye Reporter," for September 8, 1947, pages P486 to P489 inclusive.